

# UNITED STATES PATENT OFFICE.

HOMER A. BUCK, OF OAKLAND, CALIFORNIA, ASSIGNOR TO GRANVILLE MOORE, OF SAN FRANCISCO, CALIFORNIA.

## METHOD OF MAKING BINDERS FOR PIGMENTS.

1,421,125.

Specification of Letters Patent. Patented June 27, 1922.

No Drawing.

Application filed June 21, 1920. Serial No. 390,639.

To all whom it may concern:

Be it known that I, HOMER A. BUCK, a citizen of the United States, residing at Oakland, in the county of Alameda and State of California, have invented certain new and useful Improvements in Methods of Making Binders for Pigments, of which the following is a specification.

The present invention relates to the process of making a binder for pigments.

The primary object of the invention is to provide a process or method of making a binder or vehicle for pigments used in the printing arts, and relates more particularly to use with printing inks for rotogravure printing.

It is now common practice to use inks containing volatile oils or extracts such as gasoline, benzine and the like.

The present invention contemplates a water ink which will entirely dispense with inflammable materials, and obviously this will result in a decided forward step in this art.

It is now a common practice to run rotogravure presses in a basement, this being necessitated by the vibration of the presses, and basements as a rule afford inadequate ventilation, and the pressmen and employees frequently succumb from fumes of the inflammable matter contained in the inks. Again the fire risk is materially reduced by the use of water ink, it being a well known fact that many disastrous fires have occurred which have originated in these press rooms because of the fact that the static electricity generated in the press and paper have ignited the fumes of the aforesaid inflammable content of the ink.

Another benefit resulting from the use of a non-inflammable ink is the increased production made possible by high speed rotation of the presses, which is now impossible. Under present methods the rotogravure presses are operated at approximately five thousand revolutions per hour, while with this ink the same presses have been operated safely in excess of six thousand revolutions per hour.

Having reduced my invention to practice, I can state positively that a great saving has been accomplished in the use of this ink.

Although this binder, as hereinafter described, is applicable to various pigments, it has been developed in connection with finely

ground manganese ore, the preparation of which is made the subject of an application 390,638 (Serial number) for Letters Patent in the United States Patent Office filed of even date herewith.

The manganese pigment is extracted from manganese dioxide, and is usually in powder form and requires a binder to render it suitable as a printing ink. In my improved process, I use flake shellac, borax and water, as for example:

- |     |                       |    |
|-----|-----------------------|----|
| 1.  | 10% flake shellac.    | 60 |
|     | 5% powdered borax.    |    |
|     | 85% water.            | 70 |
| 2.  | 12.5% flake shellac.  | 75 |
|     | 6.25% powdered borax. |    |
|     | 81.25% water.         |    |
| 15. | 15% flake shellac.    | 75 |
|     | 7.5% powdered borax.  |    |
|     | 77.5% water.          |    |

It will be noted that, in the three examples given the proportion of shellac to powdered borax is 2 to 1, while the amount of water may be varied. Solutions made of this 2 to 1 proportion are used from 10 to 20%, while above 20% a saturated solution of borax is used instead of the borax powder to prevent the precipitation of borax crystals when the solution is cooled.

When the ingredients are assembled in the desired proportions they are heated in a steam jacketed kettle, or other suitable receptacle until a white foam appears on the surface of the solution. This is a very important step in the process.

The solution should be filtered through a fine wire screen to remove foreign particles present in the shellac.

In order to make the ink dry more slowly and to facilitate the removal or release of the pigment from the engraved cylinder, I provide an emulsified oil which is added to the binder, as for example:

- |     |                  |
|-----|------------------|
| 40% | cotton seed oil. |
| 10% | powdered acacia. |
| 50% | water.           |

Triturate oil and acacia. Add 80% of the 105 50% water and triturate. When emulsion forms add balance of water and again triturate.

Obviously other oils and suitable emulsifying agents may be employed.

By this method I have produced a non-inflammable ink of excellent qualification for rotogravure presses.

Having thus described my invention what 5 I claim as new and desire to secure by Letters Patent of the United States is as follows:—

1. A non-inflammable printing ink suitable for use on rotogravure paper consisting 10 of a pigment thoroughly incorporated in a non-inflammable binder.
2. A non-inflammable water ink suitable for rotogravure high speed printing consisting of a pigment thoroughly incorporated 15 in a non-inflammable binder containing emulsified oil.
3. A non-inflammable printing ink consisting of a pigment thoroughly incorporated in a non-inflammable binder containing 20 shellac, borax and water.
4. A non-inflammable printing ink consisting of a pigment thoroughly incorpo-

rated in a non-inflammable binder containing shellac and borax in the proportion of 1 borax to 2 shellac, and water.

25

5. A non-inflammable printing ink consisting of a pigment thoroughly incorporated in a non-inflammable binder containing shellac and borax in the proportion of 1 borax to 2 shellac and emulsified oil and 30 water.

6. A step in the method of making a non-inflammable binder for pigments consisting of subjecting a mixture of shellac, borax and water to heat until a foam appears on the 35 surface of the mixture.

7. The method of making a non-inflammable binder for pigments consisting of subjecting a mixture of shellac, borax and water to heat until a foam appears on the 40 surface of the mixture, and adding emulsified oil.

In testimony whereof I affix my signature.  
HOMER A. BUCK.